

## UNITED STATES PATENT OFFICE.

FELIX THUAUD, OF PARIS, FRANCE, ASSIGNOR OF ONE-HALF TO SOCIETE ELECTRO-METALLURGIQUES DE MONTRICHER, OF PARIS, FRANCE, A CORPORATION OF FRANCE.

## MAGNETIC STEEL HAVING A HIGH CONTENT OF SILICON.

No Drawing. Original application filed August 4, 1924, Serial No. 730,086. Divided and this application filed October 27, 1924. Serial No. 746,212.

To all whom it may concern:

Be it known that I, FELIX THUAUD, a citizen of the French Republic, residing at Paris, France, have invented certain new and useful Improvements in Magnetic Steels Having a High Content of Silicon, of which the following is a specification.

The present invention relates to a new alloy forming a magnetic steel having a high content of silicon, and a large permeability.

This application is a division of my application Number 730,086, filed Aug. 4, 1924.

It is known that the magnetic steels in use hitherto have the following composition;

|            | Per cent.    |
|------------|--------------|
| Carbon     | 0.10 to 0.20 |
| Manganese  | 0.15 to 0.30 |
| Silicon    | 1.50 to 3    |
| Sulphur    | 0.03 to 0.04 |
| Phosphorus |              |

Numerous experiments have shown that the compositions approaching this which have been mentioned do not reduce the hysteresis in sufficient proportions to enable a complete or almost complete demagnetization of the metal exposed to the action of a magnetic field. In fact the hysteresis meter indicates losses of the order of from 2 to 3 watts due to a considerable tension which becomes noticeable in the form of heat.

For reducing these losses of energy and to reduce them to a theoretical minimum there is used, according to the present invention, the following composition for steels under consideration.

|           | Per cent.    |
|-----------|--------------|
| Carbon    | 0.02 to 0.05 |
| Manganese | 0.04 to 0.07 |
| Silicon   | 3.50 to 4.20 |
| Nickel    | 0.05 to 3    |
| Titanium  | 0.05 to 1    |

The metal is prepared in an electric furnace after repeated refining and when it forms pure iron, that is to say when it comprises 0.02% of carbon and traces of manganese, of sulphur and of phosphorus there are incorporated therewith in the above proportions: 1, silicon; 2, nickel; 3, titanium.

Nickel and titanium have never been used hitherto in the manufacture of magnetic sheets. This application of these metals in the above magnetic steels constitutes one of the main characteristics of the invention.

It has for its object to determine an appreciable improvement of the quality of the products obtained; the hysteresis is reduced and decreased from a value of 3W to a value below 1.2W and the permeability of these sheets is increased by about 40%.

Having thus described my invention what I declare as new and desire to secure by Letters Patent is:

As a new article of manufacture a magnetic steel containing carbon 0.02 to 0.05%, manganese 0.04 to 0.07%, silicon 3.50 to 4.20%, nickel 0.05 to 3%, and titanium 0.05 to 1%.

In testimony whereof I have signed my name to this specification.

FELIX THUAUD.